

C. DANTSIZEN.

ELECTROLYTIC CELL AND THE PROCESS OF ELECTROLYZING METAL.

APPLICATION FILED MAR. 20, 1915.

1,190,122.

Patented July 4, 1916.

Fig.1.



Fig. 2.



Fig. 3.



Fig. 4.



Inventor:  
Christian Dantsizen,  
by *Alfred. Dan*  
His Attorney.

# UNITED STATES PATENT OFFICE.

CHRISTIAN DANTSIZEN, OF SCOTIA, NEW YORK, ASSIGNOR TO GENERAL ELECTRIC COMPANY, A CORPORATION OF NEW YORK.

## ELECTROLYTIC CELL AND THE PROCESS OF ELECTROLYZING METAL.

1,190,122.

Specification of Letters Patent.

Patented July 4, 1916.

Application filed March 20, 1915. Serial No. 15,740.

To all whom it may concern:

Be it known that I, CHRISTIAN DANTSIZEN, a citizen of the United States, residing at Scotia, in the county of Schenectady, State of New York, have invented certain new and useful Improvements in Electrolytic Cells and the Process of Electrolyzing Metal, of which the following is a specification.

10 The present invention relates to the electrolysis of an earth metal, particularly magnesium, and its object is to enable the electrolyzed metal to be obtained in relatively large masses.

15 When magnesium, or beryllium, is electrolyzed from a fused electrolyte in a cell having an ordinary carbon or iron cathode, the metal separates out in small globules which are recovered with difficulty 20 from the bath. I have discovered that when a metal cathode is used alloying very slowly with the magnesium or other metal to be electrolyzed, the electrolyzed molten metal adheres to the electrode and collects in large 25 masses.

30 In the accompanying drawings Figure 1 is a plan view and Fig. 2 a sectional view of an electrolytic cell illustrating my invention; Figs. 3 and 4 illustrate diagrammatically different arrangements of the electrodes.

35 The cell comprises a container 1 consisting of suitable inert material, such as magnesite brick. The electrolyte 2 may consist for example of a mixture of potassium chlorid and magnesium chlorid, the relative weights of the two materials at the beginning of the electrolyzing operation being preferably in the ratio of their molecular 40 weights. In some cases two or three per cent. of calcium fluorid may be added to the electrolyte with advantage. Molten magnesium has a specific gravity somewhat less than the electrolyte and hence the metal 45 separated clings to the electrode and tends to rise to the surface of the electrolyte. The cell may have a plurality of anodes 3 which may consist of conductive material inert with respect to the electrolyte, for example, carbon. The cathode 4 consists of material 50 remaining solid or unfused during the operation of the cell and the surface of the cathode consists of a material which slowly alloys with the metal to be electrolyzed.

For example, in the case of magnesium I 55 prefer to use galvanized or sherdarized iron as cathode. The exterior of the surface of such an electrode consists largely of zinc, and below this zinc layer is a layer of zinc-iron alloy of variable proportions, 60 the proportion of zinc gradually decreasing toward the inner iron base. When a suitable direct current is supplied by the conductors 5, 6 to the electrolyte in a molten state, the magnesium separates out at 65 the cathode, rapidly alloys with the exterior zinc layer and then more slowly alloys with the zinc in the layer of zinc-iron alloy until an equilibrium is reached. The molten metal wets the surface of the zinc- 70 iron alloy and hence remains attached. In place of zinc, the surface of the iron electrode may be alloyed with tin or copper. The surface alloyage with copper may be produced by dipping the iron electrode into 75 molten copper in a hydrogen atmosphere. Instead of a galvanized iron cathode, an alloy of iron and nickel containing a small percentage of nickel may be used as cathode.

80 An advantage is obtained by the use of a plurality of cathode conductors wetted by the electrolyzed metal, as globules of molten metal on one rod unite with globules on another rod to form large masses. When a plurality of rods are used the mass of accumulated molten metal which will adhere to the cathode is not only larger but remains stationary on one side of the cathode as indicated. As the electrolysis continues, the lump of magnesium 85 increases without 90 separating from the cathode until the bath has been depleted of magnesium salt and no lumps of magnesium exist in the bath which are not electrically part of the cathode. Recombination of magnesium with chlorin is 95 thus avoided.

99 The cathode 4 illustrated in Figs. 1 and 2 consists of rods placed side by side. With such an arrangement the mass of electrolyzed magnesium will usually accumulate on one side of the row of rods as illustrated. An even larger mass of molten magnesium may be accumulated by using a double row of rods 8, 9, as shown in Fig. 3, or by placing the rods to partially inclose 105 the accumulated lump of magnesium, as shown in Fig. 4. The amount of zinc which alloys with the metallic magnesium is so

extremely small it may be neglected for any of the known commercial uses of metallic magnesium.

What I claim as new and desire to secure by Letters Patent of the United States, is:—

1. An electrolytic cell for isolating metallic magnesium comprising a container, an anode inert with respect to a molten electrolyte containing magnesium compounds and a cathode remaining unfused during the electrolysis of the magnesium and having a surface layer wetted by molten magnesium.
- 15 2. The process of collecting by electrolysis metal tending to separate out in small globules, which consists in separating the metal in a fused state in contact with a cathode remaining unfused during the electrolysis and having a surface layer of a metal slowly alloying with the metal to be collected.
- 25 3. The process of isolating magnesium which consists in conducting current through a magnesium compound between a cathode consisting of iron, the surface of which is coated with zinc, and an anode.
- 30 4. An electrolytic cell comprising a container, a magnesium-containing electrolyte which is molten during operation of the cell, an anode, and a cathode consisting of material not readily alloyable with magnesium and remaining unfused during the electrolysis of magnesium, the surface of which is alloyed with zinc.
- 35 5. An electrolytic cell comprising a container, an electrolyte of fused salts containing an earth metal, an anode, and a cathode of iron in contact with said electrolyte, the surface of said cathode consisting largely of a metal other than iron wetted by a metal electrolyzable from said electrolyte.

6. An electrolytic cell comprising a container, an electrolyte of fused salts, an anode, and a plurality of unfused cathode 45 conductors in contact with said electrolyte, the surface of said conductors being wetted by the molten metal separating from the electrolyte and located so closely to each other that the metal accumulating on the 50 respective conductors will unite into a large mass clinging to the several conductors.

7. An electrolytic cell comprising a container, an electrolyte of fused magnesium salts, an anode, and a cathode of iron, having a surface layer of zinc-iron alloy.

8. An electrolytic cell comprising a container, an electrolyte of salts of magnesium, an anode, and a cathode of iron, a surface layer of which is alloyed with zinc, the outer surface consisting largely of zinc, and the proportion of zinc gradually decreasing toward the interior.

9. The process of collecting by electrolysis metal tending to separate from a fused 65 electrolyte in small globules which consists in separating said metal out at a cathode, the surface only of which is sufficiently alloyable with the metal electrolyzed to be wetted thereby, thus causing the accumulation 70 of the metal in masses on the cathode.

10. An electrolytic cell comprising a container, a molten electrolyte therein, containing a compound of a metal tending to electrolyze out in small globules, an inert 75 anode, and a cathode remaining unfused during the electrolysis, and consisting of a material alloying substantially at the surface only with the metal separated by electrolysis, thereby causing said metal to cling 80 to the cathode in large masses.

In witness whereof, I have hereunto set my hand this 18th day of March 1915.

CHRISTIAN DANTSIZEN.